

July 10, 1934.

J. G. CAPSTAFF ET AL

1,966,332

METHOD OF MAKING PHOTOGRAPHIC IMAGES IN DYED SILVER IODIDE

Filed June 2, 1932



Inventors:

John G. Capstaff & Merrill W. Seymour,

Atty.

Newton M. Perrins.

Atty.

## UNITED STATES PATENT OFFICE

1,966,332

## METHOD OF MAKING PHOTOGRAPHIC IMAGES IN DYED SILVER IODIDE

John G. Capstaff and Merrill W. Seymour,  
Rochester, N. Y., assignors to Eastman Kodak  
Company, Rochester, N. Y., a corporation of  
New York

Application June 2, 1932, Serial No. 615,032

7 Claims. (Cl. 95—6)

This invention relates to a method of making photographic images in silver iodide and particularly to a method of making color images.

It is well known that positive silver images 5 may be made by uniformly exposing a silver bromide emulsion to light, converting the silver bromide to silver iodide by means of potassium iodide solution, exposing the converted emulsion to a desired subject, and developing in a vigorous 10 photographic developer. It has also been found that, by treating the silver iodide emulsion with potassium bromide together with certain desensitizing dyes, a reversed image may be obtained.

A brief explanation will make clearer the basis 15 of the process just described and that of our invention. In order to form a developable latent image in a silver iodide and gelatin emulsion by the action of light, the presence of an iodine acceptor at the time of exposure is necessary. 20 Various substances may function in this role, among them being sodium sulfite, sodium hydroxide, and monomethyl-paramido phenol.

If, on the other hand, no acceptor is present 25 at the moment of exposure, but instead potassium iodide is in contact with the silver iodide, not only can no developable negative image be formed but any latent image which may have been present will be bleached or reversed on further exposure to light. In the method above, 30 the latent image formed in silver bromide is not destroyed when the silver bromide is converted to silver iodide. After the conversion, however, there is excess of potassium iodide present and further exposure bleaches the already 35 fogged silver salt and thus yields a positive image.

We have found that it is possible to start with 40 a silver iodide emulsion and obtain either a positive silver image or a negative silver iodide image. Our invention, briefly, is carried out as follows 45 reference being made to the accompanying drawing, in which there is shown in the form of a flow sheet the relation of the several steps of the process:

A silver iodide emulsion is bathed in a chemical sensitizer, such as a dilute solution of sodium sulphite or sodium hydroxide, dried, and uniformly exposed to a strong light. After this exposure, the plate is thoroughly washed to remove the chemical sensitizer, treated with a solution 50 of potassium iodide and dried. The plate is now exposed to a light image and developed in a powerful photographic developer. A positive silver image and a negative silver iodide image are present at this point.

55 The positive silver image may be fixed by an

ordinary sodium thiosulphate solution, or it may be removed with an oxidizing bleaching solution, leaving only the negative silver iodide image. The silver iodide image may be used to mordant 60 various basic dyes and so yield colored images by bathing in the dye solutions.

Alternatively, basic dyes may be incorporated 65 in the silver iodide emulsion at the time of making. This is done preferably by having the dye present at the time of precipitation of the silver iodide. A deeply dyed silver iodide is thus obtained. The excess of soluble salts is washed from the emulsion in the usual manner. The coated and dried plates are then treated with the chemical sensitizer as above, uniformly exposed to strong light, washed to remove the chemical sensitizer, treated with a solution of potassium iodide, dried, exposed to the desired 70 subject and developed in a powerful photographic developer.

The plate is then bleached in an oxidizing solution. At this stage it will be found that the dye has been liberated in the places where the silver iodide was reduced to silver and that a negative dye image remains adsorbed to silver 75 iodide.

Our invention makes use of the same principles as first outlined, but has certain advantages over the older method. We start with a silver iodide emulsion and sensitize it or bathe it in an iodine acceptor. This renders the silver iodide susceptible to the formation of a latent image upon exposure to light. The plate is then uniformly exposed or fogged. The sensitizer (iodine acceptor) is next washed out, and the plate bathed 80 in potassium iodide solution. The silver iodide is now in a state such that further exposure bleaches the latent image already formed to an extent dependent upon the amount of such exposure, and thereby forms a positive image on 85 exposure to a light image. The plate is developed in a powerful developer and may thereafter be treated in one of several ways.

One of the chief advantages in our invention 90 lies in the fact that basic dyes may be readily incorporated in, or mordanted to, the silver iodide emulsion at the time of making and this dye remains in the emulsion throughout the subsequent operations until the silver image is bleached.

This makes it possible to prepare several iodide 95 emulsions dyed with different colors and to mix these dyed emulsions, each kind of grain retaining its specific color sensitivity. Such mixed emulsions may then be used for a direct color process in which the grains of the different colors 100

60

65

70

75

80

85

90

95

100

105

110

are simultaneously exposed and treated by various chemical reagents.

It also makes it much more convenient to produce a monochrome image. If one starts with 5 silver bromide, fogs, converts to silver iodide and then produces the reversal image, the plate must be dyed in the later stages by a separate operation. Our invention obviates this.

In a preferred form of our invention, we proceed as follows:

A silver iodide emulsion containing a dye is made. For this we may use, by way of example, the following formula:

15 *Solution I*

|                                     |        |
|-------------------------------------|--------|
| Gelatin, 12½% solution              | 30 cc. |
| Silver nitrate, 100 grams per liter | 15 cc. |
| Basic dye, 1% solution              | 10 cc. |

20 *Solution II*

|                                       |        |
|---------------------------------------|--------|
| Gelatin, 12½% solution                | 30 cc. |
| Potassium iodide, 100 grams per liter | 17 cc. |

Solution II is poured into Solution I with vigorous 25 stirring and is made into an emulsion by methods which are well known and which include setting, shredding, washing, remelting and coating.

A large number of dyes are available for use in making this emulsion, two examples being Malachite green and Pyronine G, these dyes having 30 respectively the British Color Index numbers 657 and 739.

After plates or films coated with this emulsion are dried, they are bathed in a chemical sensitizer, 35 such as for example a ½% solution of sodium sulphite or a ½% solution of sodium hydroxide. The plates are then dried and uniformly exposed to a strong light. After exposure, the plates are thoroughly washed to remove the chemical 40 sensitizer and are then treated preferably with a 1% solution of potassium iodide. The plates are again dried. They are next exposed to the desired subject. They are then developed in a powerful photographic developer, such as what is 45 well known in the art as a caustic hydroquinone process developer. Finally, they are bleached in an oxidizing solution of which the following is a satisfactory formula:

50 Sulphuric acid, 100 grams per liter 4 cc.  
Potassium bichromate, 100 grams per liter 4 cc.  
Water to 200 cc.

It is found that the dye color-sensitizes the 55 silver iodide, both for the first or fogging exposure and for the second or image-forming exposure. Thus, Malachite green makes the silver iodide red sensitive, while Pyronine G makes it green sensitive.

Our invention may be used advantageously to 60 obtain monochrome dye images, since it requires less image-forming exposure than the process in which a negative silver image is developed from silver iodide and a positive dye image is subsequently obtained.

65 Our invention would likewise be useful in a so-called mixed grain process, it being possible to mix intimately three separate portions of silver iodide emulsions, each dyed a different color, and then to process such a mixed emulsion by the methods

70 we have given.

It is understood that our invention is not

limited by the examples given, but we contemplate as included therein all modifications and equivalents which fall within the scope of the appended claims.

What we claim is:

1. The method of producing photographic images which comprises precipitating a silver iodide emulsion, forming a layer therefrom, bathing with an iodine acceptor uniformly exposing the layer to light, treating the layer with an alkali iodide, exposing it to a light image and developing the image. 80

2. The method of producing photographic images which comprises chemically sensitizing a silver iodide emulsion layer, uniformly exposing said layer to strong light, removing any excess chemical sensitizer, treating the layer with a solution of potassium iodide, exposing the layer to a light image, and developing. 85

90 3. The method of producing photographic images which comprises chemically sensitizing a silver iodide emulsion layer, uniformly exposing said layer to a strong light, washing the layer to remove the chemical sensitizer, treating the layer with a solution of potassium iodide, exposing the layer to a light image, and developing in a powerful photographic developer. 95

100 4. The method of producing photographic images which comprises precipitating an emulsion containing silver iodide and dye absorbed to the silver iodide, forming a layer therefrom, uniformly exposing the layer to light, treating the layer with an alkali iodide, exposing it to a light image, developing a silver image in the layer and removing the silver image and the dye associated therewith, thus leaving a dyed silver iodide image. 110

115 5. The method of producing a photographic color image which comprises chemically sensitizing a silver iodide emulsion layer, uniformly exposing said layer to a strong light, washing the layer to remove the chemical sensitizer, treating the layer with a solution of potassium iodide, exposing the layer to a light image, developing in a powerful photographic developer, removing the 120 positive silver image with an oxidizing bleaching solution, and mordanting a dye to the remaining silver iodide image.

125 6. The method of producing a photographic color image which comprises chemically sensitizing a silver iodide emulsion layer, uniformly exposing said layer to a strong light, washing the layer to remove the chemical sensitizer, treating the layer with a solution of potassium iodide, exposing the layer to a light image, developing in a 130 powerful photographic developer, removing the positive silver image with an oxidizing bleaching solution, and mordanting a basic dye to the remaining silver iodide image.

135 7. The method of producing a photographic color image which comprises chemically sensitizing a silver iodide emulsion layer containing a basic dye absorbed to the silver iodide, uniformly exposing said layer to a strong light, washing the layer to remove the chemical sensitizer, 140 treating the layer with a solution of potassium iodide, exposing the layer to a light image, developing and then removing the developed image, leaving a dyed silver iodide image. 145

JOHN G. CAPSTAFF.  
MERRILL W. SEYMOUR.

**CERTIFICATE OF CORRECTION.**

**Patent No. 1,966,332.**

**July 10, 1934.**

**JOHN G. CAPSTAFF, ET AL.**

**It is hereby certified that error appears in the printed specification of the above numbered patent requiring correction as follows: Page 2, lines 105 and 138, claims 4 and 7, respectively, for "absorbed" read adsorbed; and that the said Letters Patent should be read with these corrections therein that the same may conform to the record of the case in the Patent Office.**

**Signed and sealed this 11th day of September, A. D. 1934.**

**Leslie Frazer**

**(Seal)**

**Acting Commissioner of Patents.**